

## UNITED STATES PATENT OFFICE

2,025,559

## POLYCHROMATIC PRINTING PLATE

Serge Tchetchonin, Paris, France

No Drawing. Application January 26, 1935,  
Serial No. 3,643

7 Claims. (Cl. 101—131)

This invention relates to a soluble plate used in polychromatic printing and forms a continuation in part of the invention disclosed in a co-pending application titled Process for polychromatic reproduction, Serial No. 609,994, filed May 7, 1932. More particularly this invention provides a printing plate consisting of one or more color masses arranged in a suitable design and which may be hard, or plastic to any degree. 5 In use, either the plate or the object to be printed upon is coated with a suitable solvent and when the plate is applied to the object, the color design is transferred.

According to another feature of the invention, 15 the coloring masses used in the preparation of the printing plate may have as the base or principal ingredient, dextrin, gum-lac, artificial or natural tar, commercial gums, resins, and waxes, either singly or in compounds thereof. The color masses may carry pigments which are of the current types, and have an adequate solvent which may consist of water, steam, alcohol, or any commercial solvent, according to the nature of the main ingredient or base.

20 The desired quantities of these several coloring masses are applied by hand, by a brush, or by other suitable means, in a fluid, semi-fluid, plastic, elastic, half-hard, hard, pastel or pencil state, or the like, upon any suitable backing, in order to obtain the pattern or design to be reproduced, thus forming the printing plate.

25 By the use of the said plate, the polychromatic printing is effected in a direct manner and in a single operation, upon articles or objects of all kinds, for instance upon paper, pasteboard, fabrics, ceramic objects, etc. In this manner, the artist's production itself forms the printing plate, and this can be reproduced in any desired number of copies. The elastic plate also serves to 30 execute the printing upon objects of all forms, for instance upon vases.

An object of this invention is to provide an improved polychromatic printing plate.

Another object is to provide a polychromatic 45 plate which enables a clearer and more sharply defined print to be produced.

Still another object is to provide a polychromatic plate in which designs more fine in detail may be executed.

50 Other objects and advantages will in part be stated and in part be obvious upon examination of the following specification and claims.

In accordance with the invention, a certain number of coloring masses are prepared preferably by employing in all cases the same substance

as a base or carrier, and adding any desired coloring pigments. Such coloring masses may be, as desired, fluid, semi-fluid, elastic, plastic, half-hard, hard or the like. This state of the mass will depend upon the quantity of the solvents employed in its preparation. A fluid mass can be transformed into a plastic mass by treating it for a certain time at a determined temperature in order to eliminate the excess of solvents. 5

For the preparation of a printing plate, the 10 various masses are employed in the same manner as ordinary colors. The desired amount of each mass is placed by the brush, or directly by hand, or by any other means, upon any suitable backing or support, which may consist of paper, tissue, 15 pasteboard or the like, thus forming the pattern or design which is to be reproduced. The thickness of the layer placed upon the backing may vary at will. When the design is finished, it is dried, and may for this purpose be subjected to 20 the action of heat. This forms the printing plate which serves for the polychromatic reproduction.

The fabric, paper or the like, upon which the 25 printing is to be effected, is covered with a layer of the solvent for the mass forming the base of the said coloring masses, and the plate is then applied to the said fabric, paper or other material. The printing plate itself might be coated with the solvent, while the object remains dry. The printing 30 is rapidly effected, and without requiring the use of fixing agents, mordants or like auxiliary substances. The printing plate may have a sufficient thickness to provide for the reproduction of as many copies as desired.

The proper quantities of coloring masses used 35 on the printing plate may as above stated be placed on the latter by hand, by the brush, or in any other manner. The fluid or semi-fluid masses are put on by the brush. As concerns the plastic, elastic, half-hard, hard or other masses, 40 these are adapted to produce certain particular surface effects, such as marbled surfaces, foliated surfaces, granular surfaces, or the like. The foliated parts of the image or pattern may be preliminarily prepared by hand or by machine, and 45 optionally in molds, and may consist of superposed thin sheets of a plastic substance. The hard mass may be ground, and grains of a uniform or a variable size may be incorporated into the plastic, semi-fluid, fluid or other masses, and this will form the granular parts of the image. The marbled parts can be formed by superposing sheets of masses of different colors, and by subjecting them to a mechanical action, such as pressure, or by mixing suitable masses of various na- 50 55

tures and then rolling them into sheets, or in any other manner.

An alcohol soluble mass may have the following composition:

|    |              |     |       |
|----|--------------|-----|-------|
| 5  | Gum-lac      | 100 | grams |
|    | Soap         | 15  | grams |
|    | Linseed oil  | 15  | grams |
|    | Egg yolk     | 10  | grams |
| 10 | Naphthaline  | 4   | grams |
|    | Acetic acid  | 5   | grams |
|    | Glycerin     | 10  | grams |
|    | Alcohol, 90° | 1/6 | litre |

Any suitable pigment, even metallic, may be added in any proportion.

The method of preparation of masses of this class is as follows: The gum-lac is first dissolved in the alcohol; the total amount of the pigment, naphthaline, soap, oil and acetic acid, is then added to the gum-lac solution. The whole is boiled until it becomes sufficiently thick, and is then somewhat cooled, then adding the glycerin and heating to 60°-80° C. for a sufficiently long time, while stirring, but without any abrupt movements, in order that no air bubbles shall enter the mixture.

When the mass has reached a certain consistency, the egg-yolk previously beaten with alcohol so as to form a homogeneous mass is added. The mass is then cooled, and is ready for use.

It is often important, in order to prepare a printing plate, to dilute a color, or to employ a colorless mass upon a part of the said plate, in order to obtain reproductions of graduated tints, and regions without color. The said colorless mass may have the following compositions:

|    |                       |     |       |
|----|-----------------------|-----|-------|
| 40 | Gum-lac               | 50  | grams |
|    | White alcohol varnish | 1/4 | litre |
|    | Liquid soap           | 25  | grams |
|    | Linseed oil           | 15  | grams |
|    | Acetic acid           | 5   | grams |
|    | Talc, or potato flour | 20  | grams |

The method of preparation is analogous to that of the former coloring masses.

When the printing plate has been thus produced, the printing is performed as usual by placing said plate in the known machines, or in like manner.

50 The plate or the object which is to receive the reproduction may be covered with the solvent, by using spraying means, a roller, or in any other suitable way. It should be observed that owing to a more or less prolonged action of heat, it is possible to obtain at will a more or less elastic plate or a hard plate. The elastic plate is specially adapted for printing upon objects having a concave or a convex shape.

60 The thickness of the plate will depend upon the nature of the object on which the printing is to be effected, and upon the number of reproductions to be made. Old and hardened plates may be employed, provided they are subjected to the action of solvent vapors in order to render them elastic.

It will be apparent that many changes and modifications may be made in the invention by any one skilled in the art without departing from the scope or spirit thereof, as defined in the following claims.

Having described my invention, what I claim is:

1. A printing plate for polychromatic reproduction comprising an alcohol soluble base, a fatty body, naphthaline, and a pigment.

2. A printing plate for polychromatic reproduction which comprises ingredients in substantially the following proportion:

|                       |                  |       |
|-----------------------|------------------|-------|
| Gum-lac               | 50               | grams |
| White alcohol varnish | 1/4              | litre |
| Soap                  | 25               | grams |
| Linseed oil           | 15               | grams |
| Acetic acid           | 5                | grams |
| Talc                  | 20               | grams |
| Pigment               | desired quantity | 20    |

3. A printing plate for polychromatic reproduction which comprises ingredients in substantially the following proportion:

|                       |                  |       |
|-----------------------|------------------|-------|
| Gum-lac               | 50               | grams |
| White alcohol varnish | 1/4              | litre |
| Soap                  | 25               | grams |
| Linseed oil           | 15               | grams |
| Acetic acid           | 5                | grams |
| Potato flour          | 20               | grams |
| Pigment               | desired quantity | 30    |

4. A printing plate for polychromatic reproduction which comprises ingredients in substantially the following proportion:

|             |                  |       |
|-------------|------------------|-------|
| Gum-lac     | 100              | grams |
| Soap        | 15               | grams |
| Linseed oil | 15               | grams |
| Naphthaline | 4                | grams |
| Acetic acid | 5                | grams |
| Glycerine   | 10               | grams |
| Alcohol     | 1/6              | litre |
| Pigment     | desired quantity | 40    |

5. A printing plate for polychromatic reproduction which comprises ingredients in substantially the following proportion:

|             |                  |       |
|-------------|------------------|-------|
| Gum-lac     | 100              | grams |
| Soap        | 15               | grams |
| Linseed oil | 15               | grams |
| Egg yolk    | 10               | grams |
| Naphthaline | 4                | grams |
| Acetic acid | 5                | grams |
| Glycerine   | 10               | grams |
| Alcohol     | 1/6              | litre |
| Pigment     | desired quantity | 55    |

6. A printing plate for polychromatic reproduction comprising an alcohol soluble base, a saponified fatty substance and a pigment.

7. A printing plate for polychromatic reproduction comprising an alcohol soluble base, a saponified fatty substance, an inert filler, and a pigment.

SERGE TCHECHONIN. 65